

## UNITED STATES PATENT OFFICE

2,290,364

SURFACE TREATMENT OF ALUMINUM OR  
ALUMINUM ALLOYSMartin Tosterud, New Kensington, Pa., assignor  
to Aluminum Company of America, Pittsburgh,  
Pa., a corporation of PennsylvaniaNo Drawing. Application June 27, 1940,  
Serial No. 342,707

3 Claims. (Cl. 148—6)

This invention relates to the treatment of aluminum and aluminum alloy surfaces to produce thereon colored coatings, particularly colored coatings of a permanent light fast nature. The term "aluminum," as used herein and in the appended claims, includes this metal in every degree of purity. The term "aluminum alloys," as used herein and in the appended claims, includes all aluminum alloys having an aluminum content of 50 per cent or more.

The invention particularly relates to the coloring of aluminum oxide coatings by the precipitation of iron oxide therein. While it is apparent that iron oxide has characteristics which make it most desirable as a coloring medium for oxide coated aluminum articles, all previous efforts have failed in the coloring of oxide coated aluminum with this material. This failure is probably due to the fact that the common hydrolyzable salts of iron, namely, ferric chloride, ferric nitrate, and ferric sulfate in solution give a high hydrogen ion concentration. Efforts to adjust the hydrogen ion concentration of solutions of these salts with an alkaline material such as ammonium hydroxide invariably result in the precipitation of iron hydroxide from the solution. Actually, it has been found that almost all of the iron is removed from the solution before the hydrogen ion concentration can be adjusted to a range which will give an effective precipitation of the iron oxide in the aluminum oxide coating.

The present invention comprises a method of effecting the precipitation of iron oxide in an aluminum oxide coating. By the method of this invention a wide range of colors from light golden yellows to dark reddish browns may be produced. All of these colors are characterized by permanence, resistance to fading on exposure to light, and a pronounced resistance to weathering. The stability of the solutions utilized in the coloring step is very marked and a large number of oxide coated aluminum articles can be colored in a given solution without substantial variation in the color produced. The solutions utilized are capable of adjustment by means of the addition of an alkaline material such as ammonium hydroxide to give a hydrogen ion concentration which will be effective to precipitate iron oxide in the aluminum oxide coating being treated. A pronounced advantage of the present invention lies in the fact that the coloring of the oxide coating by means of the treatment herein described is effective in a single step operation and permits adsorption by the oxide coating.

In practicing my invention in the preferred manner the aluminum or aluminum alloy which is to be treated is first provided with an oxide coating of certain characteristics. In order that the coating will not later separate from the metal surface, it is necessary that it be hard, dense, and

adherent. Of great importance, however, is the adsorbent nature of the coating. In order to obtain the most satisfactory results the oxide coating should be adapted to adsorb a substantial amount of the solution with which, as above mentioned, it later comes in contact. A further desirable quality of the oxide coating is its thickness, a comparatively thick coating being preferable. However, the thickness of the coating is not a controlling factor, and some comparatively thin coatings, artificially produced, will give good results. Being adsorbent, the coating is necessarily porous.

According to the present invention and as the first part thereof, the aluminum or aluminum alloy article is treated to produce upon its surface an oxide coating which is hard and dense and which has adequate adsorptive capacity for retaining the coloring agent. The term "oxide coating," as used herein and in the appended claims, is a well known designation of the art which describes a layer of aluminum oxide artificially produced on the aluminum or aluminum alloy surfaces by treatment of the metal surfaces with acids, such as sulfuric, chromic, etc., or alkalies, such as sodium carbonate or the alkali sulfates and acid sulfates such as sodium sulfate or sodium acid sulfate, etc., all with or without the addition of other substances and some with and some without the use of externally-applied electrical energy. The term "oxide coating" does not include the very thin film of aluminum oxide which is naturally formed upon that metal or its alloys by reason of contact with the air.

The manner in detail of producing oxide coatings on aluminum and aluminum alloys having the above described characteristics is well known and sufficiently described in the art, and consequently only preferred solutions and methods will be specifically described. The coatings which have been found to give the best results are the anodic coatings produced in oxalic acid solutions containing from 3 to 10 per cent oxalic acid, anodic coatings produced in chromic acid solutions containing from 3 to 10 per cent chromic acid, and anodic coatings produced in sulfuric acid solutions containing from 1 to 70 per cent sulfuric acid. The preferred anodic coating treatment is with a solution containing from 10 to 25 per cent sulfuric acid.

The present invention is predicated upon the discovery that iron oxide can be precipitated in the aluminum oxide coatings from aqueous solutions containing ferric oxalate. Suitable aqueous solutions containing ferric oxalate may be obtained by the use of ferric oxalate itself or almost any combination of materials which will give a ferric oxalate solution. Suitable solutions may be produced by the addition of soluble oxalates to solutions of the common ferric salts

such as ferric chloride, ferric nitrate, and ferric sulfate. Soluble oxalates which are particularly suitable as additions to solutions of ferric chloride, ferric nitrate, and ferric sulfate are the soluble alkali metal oxalates including ammonium oxalate. The advantages of the present invention can apparently be obtained independent of the method used for obtaining the solution of ferric oxalate.

While almost any solution containing ferric oxalate will give the advantages of the present invention, a preferred solution is prepared by the addition of a soluble alkali metal oxalate or ammonium oxalate to a solution of a soluble ferric salt in proportions which give about 1 to 3 mols of the soluble alkali metal or ammonium oxalate to 1 mol of ferric oxalate. Solutions prepared in these proportions can be used through a wide range of temperatures and concentrations to produce a wide range of colors, from light yellow to dark reddish brown, depending in part upon the temperature of the solution and the time of treatment. The hydrogen ion concentration of these solutions may be adjusted through a wide range by the addition of a suitable alkaline material such as ammonium hydroxide without any substantial loss of iron from the solution.

These solutions of ferric oxalates and alkali metal oxalates or ammonium oxalates can be effectively used in a hydrogen ion concentration range, varying from pH 2 to pH 7. The most satisfactory hydrogen ion concentration for general purposes is from pH 4 to pH 6.5, and for most purposes it is preferred to operate in a range between pH 6 and pH 6.5.

The concentration of these solutions can be varied widely to accommodate other operating conditions. Very dilute solutions and saturated solutions may be effectively employed in the process but generally the most effective results can be obtained when the ferric oxalate solution or the ferric oxalate-alkali metal or ammonium oxalate solution is in a concentration range of the ferric salt of from 3 to 20 per cent with a range of from 5 to 10 per cent preferred.

Solutions of the above concentration may be used at temperatures ranging from atmospheric to about the boiling point. The best results in the shortest time are easily obtained when the solutions are used at temperatures ranging from 120° F. to 140° F. In general it is preferable to use slightly higher temperatures when ferric oxalate-alkali metal or ammonium oxalate solutions are used than when using ferric oxalate solutions alone.

The method of treating an oxide coated aluminum article in the solutions above described consists in merely immersing the article in the solution. The time of immersion in any given solution is dependent upon the color desired. In general, the longer immersion time, the darker the color produced. Suitable examples of commercial procedures of producing oxide coated aluminum articles having ferric oxide precipitated therein are given hereinbelow. These examples are merely typical of the general procedure employed in producing satisfactorily colored oxide coated aluminum articles in accordance with the invention, and it is to be understood that the conditions employed may be varied widely as described hereinabove to obtain the characteristics desired in the product.

5

10  
15  
20  
2530  
3540  
4550  
5560  
65

70

#### Example 1

Aluminum articles are anodically coated in a 15 per cent sulfuric acid solution with a current density of 12 amperes per square foot for 60 minutes at 70° F. The articles are washed in water and then immersed in a 5 to 10 per cent ferric oxalate solution, adjusted to a pH value between 6 and 6.5 by means of the addition of ammonium hydroxide, for 20 minutes at a temperature of 122° F., then washed, dried, and, if desired, finally buffed.

#### Example 2

Aluminum articles coated as described in Example 1 are washed and immersed in a 10 per cent ferric oxalate solution to which has been added three mols of potassium oxalate for each mol of ferric oxalate, and having an adjusted pH value of from 6 to 6.5 for a period of 20 minutes at 140° F. The colored articles are then washed, dried, and buffed.

#### Example 3

Aluminum articles coated as described in Example 1 are washed and then immersed in a 5 per cent ferric oxalate solution to which 1 to 3 mols of potassium oxalate have been added for every mol of ferric oxalate. The adjusted pH value of the solution is between 6 and 6.5. The articles are immersed for a period of 20 minutes at temperatures ranging between 122° F. and 140° F. The colored articles are washed, dried, and buffed.

#### Example 4

Aluminum articles coated as described in Example 1 are washed and immersed in a solution containing from 5 to 10 per cent ferric nitrate plus 5 to 10 per cent potassium oxalate, or a solution containing 5 to 10 per cent ferric sulfate plus 5 to 10 per cent potassium oxalate, or a solution containing from 5 to 10 per cent ferric chloride plus 5 to 10 per cent potassium oxalate, respectively, for a period of 20 minutes at a temperature of 122° F. The colored articles are then washed, dried, and buffed.

It is to be understood that the invention is not to be limited to the specific details herein described, since these can be varied without departure from the spirit of the invention as defined in the appended claims.

#### I claim:

1. Method of coloring aluminum and aluminum alloy articles having on their surface an artificially produced oxide coating, comprising immersing the article in a solution containing ferric oxalate.

2. Method of coloring aluminum and aluminum alloy articles having on their surface an artificially produced oxide coating, comprising immersing the article in a solution containing ferric oxalate and a material selected from the group consisting of the soluble alkali metal oxalates and ammonium oxalate.

3. Method of coloring aluminum and aluminum alloy articles having on their surface an artificially produced oxide coating, comprising immersing the article in a solution containing ferric oxalate and a material selected from the group consisting of the soluble alkali metal oxalates and ammonium oxalate in an amount equal to about 1 to 3 mols to each mol of the ferric oxalate.

MARTIN TOSTERUD.